

May 26, 1953

W. R. STANTON

2,639,966

PROCESS FOR COATING COTTON FABRICS

Filed Oct. 18, 1950

3 Sheets-Sheet 1



FIG. I.

*Inventor  
William R. Stanton  
By his attorneys*

*Howson and Howson*

May 26, 1953

W. R. STANTON

2,639,966

## PROCESS FOR COATING COTTON FABRICS

Filed Oct. 18, 1950

3 Sheets-Sheet 2

FIG.2.



*Inventor  
William R. Stanton  
By his attorneys*

Howson and Howson

May 26, 1953

W. R. STANTON

2,639,966

PROCESS FOR COATING COTTON FABRICS

Filed Oct. 18, 1950

3 Sheets-Sheet 3

FIG.3.



FIG.4.



Inventor  
William R. Stanton  
By his attorneys

Hawson and Hawson

## UNITED STATES PATENT OFFICE

2,639,966

## PROCESS FOR COATING COTTON FABRICS

William R. Stanton, Penn, Wolverhampton, England, assignor to Textuff Limited, London, England, a British company

Application, October 18, 1950, Serial No. 190,688.  
In Great Britain January 18, 1949

4 Claims. (Cl. 8—18)

1

This invention relates to the coating of fabrics with cellulose. This application is a continuation in part of my application No. 136,687, now abandoned.

It is known to pass a textile fabric, which may be woven or knitted, through an aqueous bath of cellulose derivative, for example viscose, so that the fabric becomes coated with viscose, and then to treat the coated fabric with a coagulating agent which regenerates the cellulose in the viscose so that a fabric coated with cellulose is obtained. Cellulose derivatives such as viscose which can be treated to obtain cellulose are hereinafter referred to as "regeneratable cellulose derivatives." It is also known to treat the fabric before the coating operation with a view to reducing the amount of air absorbed by the fabric; thus in British specification No. 306,586, it is proposed to remove the air in the fabric before the fabric reaches the coating liquid, by passing the fabric through a vacuum chamber immediately above the surface of the liquid.

British specification No. 611,275 describes and claims a process for coating a knitted or woven fabric with cellulose by passing the fabric through an aqueous bath of regeneratable cellulose derivative and then treating it with a coagulating agent, wherein the fabric is treated with live steam immediately prior to its immersion in the coating bath in order to eliminate or to reduce to a minimum absorbed air and hence the occurrence of air bubbles or pin-holes in the final product.

In carrying out the process according to the said British specification No. 611,275 it is found that pin-holes may still sometimes result from incomplete wetting of the fabric in the viscose bath when gases arising from the decomposition of the viscose lead to the formation of bubbles or pin-holes in the final product. Furthermore, there is a marked tendency for minute blisters or protuberances, as distinct from pin-holes, to be formed on the product.

It is the object of the present invention to eliminate these further imperfections.

The present invention comprises a process for coating a knitted or woven fabric with cellulose by treating the fabric with live steam in order to eliminate or reduce to a minimum absorbed air in the fabric, treating the steamed fabric in an aqueous bath, preferably a hot aqueous bath, so that the fabric is uniformly wetted out, passing the fabric through a bath of a regeneratable cellulose derivative, treating the coated fabric with a coagulating agent and, during the coating operation, continuously withdrawing part of the

2

bath of regeneratable cellulose derivative, passing the withdrawn bath through at least one filter and continuously returning the filtered bath to the coating bath. The treatment of the steamed fabric with the aqueous bath may conveniently be effected by passing the fabric through a hot water bath with the aid of guide rollers suitably placed for guiding the fabric through the bath; after withdrawal from the bath, the fabric may be placed between squeeze rollers to remove excess water and to smooth the fabric which is then passed directly into a bath of a regeneratable cellulose derivative. The treatment of the fabric with live steam followed by the wetting out treatment serves to eliminate substantially completely the formation of pin-holes in the final product.

Investigations which I have carried out have shown that the blisters in the final product are due to fibrils of the cotton or other material of the fabric; viscose tends to coagulate on these fibrils and the aggregated viscose adheres to the fabric and appears in the final product as minute protuberances or blisters. I have found that these blisters may be eliminated or considerably reduced by continuously circulating part of the viscose bath through one or more filters during the coating operation, the filters serving to remove the fibrils of cotton and the like. Filters consisting of metal screens or fabrics having 15 to 25 holes per inch are particularly suitable for use in the filtering operation.

The fabric, after the treatment with a hot aqueous bath in accordance with the invention, may be cooled, by passing it through the air for a distance of say six feet, and so allowing some of the water to evaporate, or by subjecting it to a cold water spray, and then passed into the bath of viscose or other regeneratable cellulose derivative. The coating bath is preferably divided by suitably placed vertical grids into three or more compartments in which the grids help to restrain physically any bubbles, fibrils, aggregated fluff from the fabric or coagulated particles formed in the bath and so keep them away from the jet through which the fabric leaves the bath. The bath is preferably withdrawn from the compartment nearest the jet and, after filtering, returned to the same compartment. The viscose bath may be cooled for example by means of water at ordinary temperature (15 to 25° centigrade) or by cooled brine circulating in pipes submerged in the bath. Cooling the viscose in this way tends to limit the "aging" of the viscose which otherwise results from the heating of the viscose by the heated fabric passing through the bath.

The aqueous bath preferably contains a wetting agent such as a sulphonated long chain fatty alcohol in order to improve the wetting out of the fabric.

The aqueous bath may also contain a dyestuff which is substantive to the material of the fabric so that the fabric is coloured after the steaming treatment. In this case the viscose or other regeneratable cellulose derivative bath may be pigmented preferably so that the coating will have the same colour as the fabric; examples of dyes suitable for use with cotton are the water-soluble dyes which are resistant to both alkali and acid and are so unaffected by either the caustic soda in the viscose or the acid used as the coagulating agent. Chlorazol Sky Blue FF (Colour Index No. 518) and Diphenyl Red 7 BL (Colour Index No. 278) are specific examples of such dyes. The aqueous bath may conveniently contain from 0.1 to 0.2 per cent by weight of the dye.

The viscose used in the present invention is preferably a normal viscose as used for thread-making, that is viscose containing about 7 to 8 per cent of cellulose and about 6 to 7 per cent of caustic soda.

The knitted or woven fabric used in carrying out the present invention may be made from natural fibre such as cotton fibres or from synthetic fibres such as regenerated cellulose fibres, particularly viscose rayon fibres.

The present invention is illustrated by way of example in the accompanying drawings in which

Figure 1 is a schematic representation of the steps in the process for producing a cellulose-coated fabric.

Figure 2 is a vertical section through the steam chamber wetting out bath and viscose coating bath of the apparatus shown in Figure 1 but on a larger scale,

Figure 3 is a vertical section through the filtering apparatus for circulating the viscose bath, also on a larger scale, and

Figure 4 is a section on the line 4—4 of Figure 3 but with only one of the tubes sectioned.

Referring to Figure 1, a fabric 1 is first passed through a steam chamber 2 into a bath 3 containing a wetting-out solution 4 and the wet fabric is then led into a bath 5 containing viscose or other regeneratable cellulose solution 6. The solution 4 may contain a dyestuff for the fabric 1 and the cellulose solution 6 may contain a pigment. The coated fabric leaves the bath 5 through an adjustable slot 7 and is passed by means of a stenter 8 through an acid coagulant bath 9. It is then washed free from acid in a water bath 10 and passed on a second stenter 11 through a drier 12. Knives 13 then cut off the selvedges and the finished fabric is collected as a roll 14. Throughout the operation, part of the solution 6 is continuously circulated by a pump 15 first through a screen filter 16, then through a cloth filter 17 and finally back to the bath 5.

Referring to Figure 2, the fabric 1 enters the steam chamber 2 through a slit 18 and both sides of the fabric are sprayed with steam from two parallel rows of steam jets 19, 20. The steamed fabric leaves the steam chamber 2 through a second slit 21 and is passed into the wetting-out solution 4, under rollers 22, 23 out of the bath and between mangle rollers 24 and then down to a spreading roller 25 just above the solution 6. The spreading roller 25 is of known construction with a diameter greater in the centre and tapering away towards each end, and keeps the wet fabric from crumpling. The fabric passing from

the spreading roller 25 enters the solution 6 and is passed by means of rollers 26, 27, 28 to the nip of a pair of rollers 29, 30 and thence horizontally through centralising rods 31 to the exit slot 7

5 for further treatment as described with reference to Figure 1. The bath 5 is provided with four wire screen 32, 33, 34, 35 held in slots on the side of the bath 5; each screen conveniently has sixteen holes to the inch. The screens 32, 33, 34, 35, divide the bath 5 into three interconnected compartments 37, 38, 39. From the compartment 39, the solution 6 is circulated continuously through the filter 16, the pump 15 and the filter 17 and back to the compartment 39 by way of a pipe 40.

10 15 The filter 16 is conveniently a wire gauze filter basket 41 (Figure 3) having sixteen holes to the inch. The filter 17 consists of an outer casing 42 with a top cover 43 in which are secured seven separate filter tubes 44 each of which communicate with a space 45 above the cover 43. The tubes 44 conveniently consist of an inner perforated tube 46, a wire gauze 47 having sixteen holes to the inch wrapped around the tube 46 and a fabric filter 48, consisting of an unbleached

20 25 strainer canvas having twenty-two holes per inch, wrapped round the gauze 47. The viscose is forced upwards through the filter tubes 44 into the space 45 and thence back via pipe 40 to the bath 5.

30 35 40 In order to permit the passage of slubs through the slot 7 a counter-balancing weight 49 is provided, the weight being so adjusted that while a slab in the fabric 1 can lift the top part 50 of the jet to enable the slab to pass through, the slot 35 will immediately revert to the predetermined width once the slab has passed.

The solution 6 may be cooled by means of a water jacket (not shown) around the bath 5 or by passing a brine solution through pipes (not shown) within the bath 5.

45 50 The invention is illustrated by the following examples in which apparatus as described in Figures 1 and 2 was used.

Percentages are by weight.

#### Example 1

The wetting out solution used was a 0.15 per cent aqueous solution of Diphenyl Red 7 BL at 80° centigrade, the solution containing 0.01 per cent of a sulphonated long chain fatty alcohol as a wetting agent.

55 60 65 The viscose used contained 7.5 per cent of cellulose and 6.25 per cent of caustic soda, was aged to a salt figure of 4.0, was pigmented with 9 per cent of Monolite Fast Red 2 RVS (page 173 of "Pigments" by J. S. Remington, published by Leonard Hill, Ltd.) and 3 per cent of titanium dioxide based on the weight of the cellulose, and contained 0.15 per cent by weight, based on the weight of the cellulose, of a sulphonated long chain fatty alcohol. The temperature of the viscose bath was maintained at approximately room temperature (20° centigrade). During the coating operation, viscose was continuously circulated through a sixteen mesh basket sieve and a twenty-two mesh unbleached strainer canvas as described above with reference to the drawings.

70 75 The product was an all-red cellulose-coated fabric.

#### Example 2

The wetting out solution used was a 0.15 per cent aqueous solution of Diphenyl Brilliant Blue FF (Colour Index No. 518) at 80° centigrade, the

solution containing 0.01 per cent of a sulphonated long chain fatty alcohol as a wetting agent.

The viscose used was the same as that used in Example 1 except that the Monolite Fast Red 2 RVS and titanium dioxide pigment mixture was replaced by a mixture of 4 per cent of Irgalite Blue KRV (Geigy Chemical Company) and 4 per cent of titanium dioxide based on the weight of the cellulose.

An all-blue cellulose-coated fabric was obtained.

*Example 3*

The solution used was a 0.15 per cent aqueous solution of Chlorazol Green GS (Colour Index No. 594) at 80° centigrade, the solution containing 0.01 per cent of a sulphonated long chain fatty alcohol as a wetting agent.

The viscose used was the same as that used in Example 1 except that the mixture of pigments used contained 4 per cent of Monastral Fast Blue BVS (Journal of the Society of Dyers and Colourists, 1943, page 223), 5 per cent of Monolite Fast Yellow GNVS (Journal of the Society of Dyers and Colourists, 1943, page 223), 8 per cent of titanium dioxide and 0.25 per cent of carbon black, based on the weight of the cellulose.

An all-green cellulose-coated fabric was obtained.

What I claim is:

1. A process for coating a cotton fabric with cellulose which comprises treating the fabric with live steam in order to remove absorbed air in the fabric, passing the steamed fabric through an aqueous bath containing a wetting agent suitable for wetting out cotton so that the fabric is uniformly wetted out, passing the wetted fabric through a viscose bath, treating the viscose-coated fabric with a coagulating agent, and, during the coating operation, continuously withdrawing part of the viscose from the bath, passing the part so removed through at least one filter to remove the fibrils of cotton in the viscose, and continuously returning the filtered viscose to the coating bath.

2. A process as claimed in claim 1 in which the aqueous wetting out bath is heated and the wetted fabric is cooled before it is passed into the viscose bath.

3. A process for coating a cotton fabric with cellulose which comprises treating the fabric with live steam in order to remove absorbed air in the fabric, passing the steamed fabric through an aqueous bath containing a wetting agent suitable for wetting out cotton and at least one water-soluble direct cotton dyestuff substantive to the material of the fabric, so that the fabric is uniformly wetted out and dyed in the bath, passing the wetted dyed fabric through a viscose bath containing at least one pigment, the dyestuffs and the pigments being so selected that the cellulose coating has the same colour as the dyed fabric, treating the viscose-coated fabric with a coagulating agent, and, during the coating operation, continuously withdrawing part of the viscose bath, passing it through at least one filter to remove the fibrils of cotton in the viscose and continuously returning the filtered viscose to the coating bath.

4. A process for coating a cotton fabric with cellulose which comprises treating the fabric with live steam in order to remove absorbed air in the fabric, passing the steamed fabric through an aqueous bath containing a sulphonated long chain fatty alcohol wetting agent so that the fabric is uniformly wetted out, passing the wetted fabric through a viscose bath, treating the viscose-coated fabric with a coagulating agent, and, during the coating operation continuously withdrawing part of the viscose bath, passing it through at least one filter to remove the fibrils of cotton in the viscose and continuously returning the filtered viscose to the coating bath.

35 WILLIAM R. STANTON.

References Cited in the file of this patent

UNITED STATES PATENTS

|    | Number    | Name     | Date          |
|----|-----------|----------|---------------|
| 40 | 1,942,383 | Dickhaut | Jan. 2, 1934  |
|    | 2,378,186 | Clark    | June 12, 1945 |

FOREIGN PATENTS

|    | Number  | Country       | Date          |
|----|---------|---------------|---------------|
| 45 | 280,262 | Great Britain | Nov. 15, 1927 |
|    | 611,275 | Great Britain | Oct. 27, 1948 |